

1,164,965.

H. S. SMALLEY.  
ASPHALT ROOFING.  
APPLICATION FILED OCT. 21, 1912.

Patented Dec. 21, 1915.

FIG. I.



FIG. II.



Witnesses  
John C. Berger.  
James H. Bell.

Inventor  
Harvey S. Smalley  
by J. Wiley & Sons  
Attorneys

# UNITED STATES PATENT OFFICE.

HARVEY S. SMALLEY, OF BOUND BROOK, NEW JERSEY, ASSIGNOR TO THE BARBER ASPHALT PAVING COMPANY, OF PHILADELPHIA, PENNSYLVANIA, A CORPORATION OF WEST VIRGINIA.

## ASPHALT ROOFING.

1,164,965.

Specification of Letters Patent. Patented Dec. 21, 1915.

Application filed October 21, 1912. Serial No. 726,860.

To all whom it may concern:

Be it known that I, HARVEY S. SMALLEY, of Boundbrook, in the county of Somerset and State of New Jersey, have invented certain new and useful Improvements in Asphalt Roofing, whereof the following is a specification, reference being had to the accompanying drawings.

My invention has for its object to provide asphalt roofing sheets with a surface capable of receiving and retaining a smooth coat of paint.

Difficulty has long been experienced in the effort to paint asphalt and other bituminous roofings because of the fact that roofing felt when saturated with or coated with a bituminous cement presents a surface which is uneven and one to which paint does not adhere, so that the painted surface is neither smooth nor permanent, but tends to peel or blister off. Many efforts have been made to solve this problem. I have discovered a solution which is dependent upon the interposition between the roofing sheet and the paint of a comparatively thin sheet of ordinary paper. The presence of this sheet of ordinary paper upon the surface of the roofing felt does not interfere with its desired qualities as a roofing material, while at the same time it affords a smooth surface which readily takes and retains paint.

In the accompanying drawings, I have illustrated a simple form of roofing embodying my invention, in which—

Figure I, is an enlarged perspective view with the layers successively cut away and Fig. II, is a sectional view. In these drawings the thickness of the paper and paint layers are necessarily exaggerated.

I have illustrated the roofing proper as composed of a single sheet of roofing felt 1, but it is obvious that various other compound sheets may with similar advantage be used in connection with my invention. The main roofing sheet 1, consists of roofing felt which has been saturated by asphalt fluxed with oil. Upon the side of this roofing sheet there is applied a sheet of moderately thin ordinary paper 2. This sheet prior to its application is similarly saturated with a compound consisting of asphalt and oil for example Trinidad asphalt and

Trinidad asphaltic oil. The two sheets thus saturated are united by a heavier asphaltic cementing medium which adheres tenaciously 55 to the roofing sheet and also to the saturated paper, entering the pores thereof, and becoming more or less incorporated therewith, but not passing completely through it, or modifying the paint-receiving capacity of 60 the outer surface of the paper. Upon the outer surface of this paper sheet a layer of ordinary paint 3, may be applied. The paint enters into the interstices of the paper becoming more or less incorporated therewith, 65 and the incorporated particles of the paint commingle with those of the asphaltic cement upon the other side of the paper. The paint thus applied is firmly adherent and does not peel or blister, and owing to the 70 smooth surface of the paper, gives the roofing sheet a clean smooth painted surface with the appearance of painted wood or tin.

It will be understood that according to my invention, the sheet of paper does not necessarily add to or form an essential structural part of the roofing felt which may be considered as complete in itself. The paper is only a medium interposed between the paint and the roofing sheet in order that the 80 two may be inseparably combined, thus overcoming the difficulties which as explained occur when the paint is applied directly to the roofing sheet.

The paper should be thin enough not to add materially to the thickness of the roofing sheet, of a fine enough texture to present a smooth surface. It should be sufficiently absorbent to permit of partial incorporation with its substance of the asphaltic 90 cement applied upon the one side, and the paint upon the other, and on the other hand it should not be so open or porous as is a textile fabric. Such a textile fabric absorbs so much asphaltic cement as to allow 95 the asphaltic cement to completely penetrate it, thereby defeating the object which the present invention has in view, for the asphaltic cement which has penetrated a textile fabric affords no better surface for the 100 application of paint than the surface of the roofing sheet and for the same reason.

Having thus described my invention, I claim:

A bituminous roofing sheet having an adhering sheet of paint receiving paper cemented to the roofing sheet by an asphaltic cement, which does not so far penetrate the paper as to modify the paint receiving capacity of its outside surface.

In testimony whereof, I have hereunto

signed my name at Maurer, N. J. this 18th day of October 1912.

HARVEY S. SMALLEY.

Witnesses:

ALBERT J. HOLLOWBACH,  
M. S. DARROW.